

Dec. 21, 1937.

F. P. ROMANOFF

2,103,119

NONCORRODIBLE OBJECT AND METHOD OF PRODUCING SAME

Filed April 23, 1936

Fig. 1.



Fig. 2.



Fig. 5.



Fig. 6.



Fig. 3.



Fig. 4.



Inventor:

Frank P. Romanoff

By: Wilson, Dowell, McCann & Foley  
Attn:

## UNITED STATES PATENT OFFICE

2,103,119

NONCORRODIBLE OBJECT AND METHOD OF  
PRODUCING SAMEFrank P. Romanoff, Chicago, Ill., assignor to  
Apollo Metal Works, Chicago, Ill., a corporation  
of Illinois

Application April 23, 1936, Serial No. 75,921

## 1 Claim. (Cl. 148—6)

This invention relates to metallic objects and more particularly to objects fabricated from normally corrodible sheet metal, the purpose of the invention being primarily to produce a sheet metal object having those surfaces which are exposed to view plated and those surfaces not so exposed protected against corrosion by a rust-proofing coating.

Many articles of commerce and use are fabricated from lightweight sheet metal which, for the sake of appearance and durability of the finished article, is coated before fabrication with a non-corrodible metal such as nickel, chromium, or the like, such coatings being applied by the usual electro-plating process.

The fabrication of such sheets into the finished articles, however, usually involves piercing or penetration of the plated sheet by cutting or stamping the same to shape, and often by cutting, punching, or stamping holes or slots or slits in the sheet. After being pierced in this manner the sheets are then formed by bending operations into the desired shape of the finished object. The cutting, punching, or other piercing operations performed upon the sheets results in the exposure along or around the edges of the cuts of the raw metal of the sheet between the plated surfaces. Sometimes also the stretching of the plated sheets by the drawing or bending operations cracks or breaks the surface plating so as to expose the underlying sheet metal. In time these exposed surfaces corrode or oxidize so as to present an unsightly appearance and in some articles, even though such corroded edges or the metal where the plating has become separated may not be exposed to view, the corrosion may stain and discolor other portions of the assembly of which the fabricated sheet metal object is a part, or may result in injury by discoloration or otherwise to other articles or objects with which the corroded surfaces may be brought in contact.

This objectionable corrosion of the exposed edges or portions of articles fabricated from pre-plated sheet metal has heretofore constituted a deterrent to the use of such pre-plated sheets in the production of many articles for which such sheets would otherwise be highly desirable. Attempts have been made to overcome the difficulty by fabricating the articles from unplated metal sheets and subsequently plating the completed article, but the time and expense involved in plating articles already fabricated to shape as compared with pre-plating the metal in sheet form is so great as to practically preclude this

practice. The purpose of my present invention is to enable the fabricator of the sheet metal articles or objects to fabricate them from pre-plated metal sheets in the usual manner and then to economically render the metal surfaces exposed by the fabrication steps non-corrodible so that no portion of the completed article will thereafter be subject to corrosion.

The cost of rendering the completed sheet metal objects proof against corrosion being a highly important factor in their commercial production, my invention aims to render such objects non-corrodible in a very expeditious and economical manner so that my method can be practiced to secure the desired results without material increase in the cost of production of the objects so treated.

In addition to the type of articles above mentioned, the fabrication of which involves the piercing of the metal sheet, there are other types of articles the fabrication of which involves only bending operations without piercing or materially stretching the sheet. For the production of many of these, a metal sheet plated on one face only would meet the requirements provided the opposite face of the sheet were not subject to corrosion. Heretofore, however, in order to insure against corrosion of the concealed surfaces in the fabricated article, as well as to prevent corrosion of the exposed surface and render such exposed surface attractive in appearance, the plating of all surfaces at considerable expense has been considered necessary.

Another purpose of my invention, therefore, is to reduce the cost of production of articles of this character by eliminating the plating of that surface of the sheet which becomes concealed in the completed fabricated object, while at the same time rendering such concealed surface non-corrodible, by a method much cheaper than plating. This purpose is accomplished in accordance with my invention by plating one surface only of such a sheet and subjecting the unplated surface to the action of a corrosion resistant agent which renders such surface non-corrodible without in any way injuring or diminishing the effectiveness or appearance of the previously plated surface.

Other objects and advantages of my invention will be readily appreciated as the same becomes better understood by reference to the following description when considered in connection with the accompanying drawing.

Referring to the drawing,

Fig. 1 is a perspective view of a metal sheet, all exposed surfaces of which have been plated;

Fig. 2 is a perspective view of the sheet of Fig. 1 after it has been subjected to a piercing fabricating operation;

Fig. 3 is a fragmentary sectional view on an enlarged scale through the sheet of Fig. 1;

Fig. 4 is a similar view through the fabricated sheet of Fig. 2;

Fig. 5 is a sectional view illustrating two metal sheets contiguously arranged so that when electro-plated the metal coating is applied to one face and the edges only of each sheet, as illustrated; and

Fig. 6 is a similar view of one of the sheets shown in Fig. 5 after it has been subjected to the action of a rustproofing agent.

It should be at once noted that in the illustrations on the accompanying drawing the thickness of the sheets, and also the coatings thereon, are greatly exaggerated. While my invention, of course, is applicable to sheets of almost any thickness, its most profitable field of commercial utility is found in connection with articles made from relatively light gauge sheet metal.

In carrying out my improved method in accordance with the disclosure of Figs. 1 to 4, inclusive, a metal sheet of any desired size and thickness is first subjected to an electro-plating operation by which all exposed surfaces, including both faces and the edges of the sheet, are electro-plated with the desired metal, such as chromium or nickel, for instance. Such a sheet is indicated in Fig. 1 of the drawing by reference character 7, and the metal coating applied to the surface thereof, commonly termed plating, is indicated in Fig. 3 by reference character 8. Such plated sheets are sold by the manufacturer thereof to the fabricator, who shapes and forms them into the desired objects by fabrication processes which usually include not only operations which bend the sheet into form but also operations which involve piercing the sheet by cutting, punching, stamping, or other similar operations. For illustrative purposes the partially fabricated sheet shown in Fig. 2 has been subjected to cutting operations which removed two of the corners, leaving exposed edges 9 and 11 and also provide perforations 12, the walls of which present exposed metal surfaces between the plated surfaces of the sheet.

It will be obvious that if such a cut and punched sheet were now formed by bending operations into a completed article, such article would present unplated surfaces where the cutting and punching was performed which would be subject to corrosion. In accordance with my invention these exposed metal surfaces are made rustproof or non-corrodible by subjecting them to the action of a rustproofing or corrosion resistant agent which causes the formation of a coating of non-corrodible phosphate upon these exposed surfaces without in any way injuring or affecting the plated surfaces of the sheet.

This rustproofing operation may be performed either immediately after the sheet has been cut and punched or after it has been bent and formed into the shape of the finished object; but preferably for convenience in handling, the rustproofing is done after the bending or forming operation.

While various solutions may be utilized for producing the desired rustproofing effect, the preferred rustproofing coating comprises a chemical which has a phosphate base resulting in the formation of a phosphate coating on exposed surfaces of the sheets subjected to such solution.

The coating operation is purely a chemical action which takes place readily when the object is submerged in a bath containing the coating solution. For instance, the solution may contain manganese phosphate which chemically reacts with the steel or similar metal of the sheet to form a coating of phosphate of iron on the exposed surface of the sheet. Satisfactory results may also be obtained by submersion of the article to be coated in a phosphoric acid bath, and there are also available various soluble powders comprising phosphate compounds adapted when in solution to chemically react upon the exposed metal surfaces of the object to be coated to deposit upon such surfaces a rustproof phosphate coating.

As previously stated, the chemically created phosphate coating is readily formed upon the exposed surfaces so that the time required for submersion in order to produce an average coating is not excessive. Since the solution itself is not expensive to produce the entire cost of the method both as to time and materials is moderate so that the method may be very economically practiced.

Some articles and objects, as previously stated, require the metal sheet from which they are formed to be plated on one face only, and for the production of sheets for this purpose my invention may also be utilized. In the accomplishment of this purpose the sheets, instead of being plated on both faces, are placed in pairs in the electro-plating bath with their opposed faces in contiguous relation. Such an arrangement of the sheets is illustrated in Fig. 5, wherein the sheets 12 and 13 are disposed face to face and in this position subjected to the plating operation which deposits a coating 14 on the outer faces and edges only of the sheets, leaving the contiguously disposed faces unplated. After being plated the sheets are then separated and immersed in the corrosion resistant bath which results in the formation of a non-corrodible coating 15 on the unplated surface of the sheet. The resultant sheet accordingly has a corrosion resistant coating on one face and is plated on the opposite face and on the edges, so that all of the surfaces are covered and protected. Such sheets are suitable for fabrication without further coating treatment in the production of those articles or objects the fabrication of which does not require any piercing or penetration of the sheet. For some purposes a sheet plated on both sides with the edges unplated but rendered corrosion resistant is desirable. My invention is obviously suitable for the production of such sheets also.

The details of the method which has been described as illustrative may obviously be varied within considerable limits within the scope of the invention as defined in the following claim.

I claim:

The method of making a non-corrodible sheet metal article which comprises producing by electrolytic deposition upon the exposed portions of a metal sheet a metal coating resistant to attack by a rustproofing phosphate base solution, fabricating the thus electroplated sheet to form an article of the desired shape in which portions of the base metal of the fabricated sheet are left exposed, and rustproofing said exposed portions without affecting the previously electroplated portions of the article by immersing the article in a rustproofing phosphate solution.